

March 3, 1936.

S. RUBEN

2,032,439

ELECTRIC CURRENT RECTIFIER

Filed April 13, 1933



INVENTOR

*Samuel Ruben*

Watson, Bristol, Johnson & Leavenworth  
ATTORNEY

## UNITED STATES PATENT OFFICE

2,032,439

## ELECTRIC CURRENT RECTIFIER

Samuel Ruben, New Rochelle, N. Y., assignor to  
 Ruben Rectifier Corporation, Englewood, N. J.,  
 a corporation of Delaware

Application April 13, 1933, Serial No. 665,869

9 Claims. (Cl. 175—366)

This invention relates to electric current rectifiers and the like which employ asymmetric or unilateral conductive couples of the dry surface-contact variety, the term "unilateral conductive couple" as used hereinafter being intended to designate a device including an electrode element of a relatively electropositive material and another electrode element of a relatively electro-negative material adapted to cooperate with the former for the electrochemical formation and maintenance at their junction of an inverse current-blocking film which has the property of conducting current in one direction and blocking current in the reverse direction.

General objects of the invention are the provision of such couples having improved characteristics, which are efficient, economical and readily manufactured, and have long service lives; the provision of an additional element in such couples which tends to prevent in operation the formation of polarizing material of a character which reduces the efficiency and shortens the service life; and structural embodiments of the device which are readily constructed and allow efficient use and operation thereof.

A specific object of the invention is the provision of such a couple provided with a layer of non-polarizing substance in contact with the material constituting the electronegative electrode element thereof to prevent the formation in operation of polarizing material adjacent the electro-negative material, and to insure steadiness of output and increased efficiency.

Another object of the invention is the provision of such a unilateral conductive couple wherein the electropositive electrode element is composed of a relatively electropositive material formed from one of the elements chosen from an empirical group including beryllium, magnesium, calcium, zinc and aluminum, or alloys or compounds thereof, and the other electrode element is composed of a relatively electronegative material, preferably including at least one compound of at least one of the elements sulphur, selenium, and tellurium, the couple additionally being characterized by a layer of a non-polarizing substance interposed between the electronegative material and a terminal member.

A further object of the invention is the provision in such a unilateral conductive couple having an electropositive electrode of a silicon material having a high contact resistance with the electronegative electrode element and preferably formed from a silicide compound of one of the elements chosen from an empirical

group including beryllium, magnesium, calcium, zinc and aluminum, with the electronegative electrode element formed of a material preferably including at least one compound of at least one of the elements sulphur, selenium and tellurium, of a welded junction obtained by subjecting the electropositive and electronegative materials to a flow of electric current to weld them together to form a physically and electrochemically stable unitary couple element.

Other objects of the invention will in part be obvious and will in part appear hereinafter.

The invention accordingly comprises the features of construction, combination of elements and arrangement of parts which will be exemplified in the following detailed disclosure, and the scope of the application of which will be indicated in the claims.

For a fuller understanding of the nature and objects of the invention reference should be had to the following detailed description taken in connection with the accompanying drawing, in which:

Fig. 1 is a sectional schematic view of an empirical unilateral conductive couple of the dry surface-contact variety formed in accordance with the present invention;

Fig. 2 is a sectional view of one structural form of the device of the present invention utilizing couples of the type depicted in Fig. 1;

Fig. 3 is a sectional view of a structural modification on the device of the present invention;

Fig. 4 is a top plan view with parts in section and parts broken away of a further structural modification of the device of the present invention;

Fig. 5 is an end view of the device depicted in Fig. 4; and

Fig. 6 is a sectional view of one of the couple units of the structure depicted in Figs. 4 and 5.

Prior to the present invention electric current rectifiers and the like which employed asymmetric or unilateral conductive couples of the dry surface-contact variety have been provided with an essential contact resistance between the electropositive and electronegative electrode elements in a variety of ways. These devices, at times, have been characterized by non-uniform operating characteristics, instability during operation under ordinary atmospheric conditions, and have had relatively short service commercial lives. These and other undesirable characteristics are substantially avoided by the present invention.

In accordance with the present invention a device of this type is provided which has an elec-

- tropositive electrode element formed from a relatively electropositive material of a chemical element or compound thereof, provided if desired with a surface coating of another compound of 5 relatively electropositive material. Some of the chemical elements which have been found to be suitable are beryllium, magnesium, calcium, zinc and aluminum. Relatively electropositive alloys of such elements may also be used, for example, 10 an alloy of silicon with one of the above metals, aluminum with magnesium, and amalgams of aluminum and magnesium.
- The electronegative electrode element is formed from a relatively electronegative material such 15 as a metallic compound or mixture of compounds of elements chosen from an empirical group of elements of Sub-group B of the Sixth Periodic Group in Mendeleeff's Periodic Table of Elements, for example, oxides, sulphides, selenides 20 and tellurides. Some of the metallic elements from which it has been found suitable to form these compounds are copper, silver, cadmium, mercury, zirconium, lead, vanadium, arsenic, antimony, tantalum, bismuth, chromium, bolybdenum, tungsten, manganese and iron. Alloys 25 of copper, such as brass, bronze and copper with any of the elements zinc, silver, lead, tin antimony, etc., have also been found suitable from which to form the oxides, sulphides, selenides or 30 tellurides. In addition, mixtures of the compounds, such as mixtures of oxides of various of the above mentioned metals, mixtures of sulphides and selenides or tellurides, and mixtures 35 of one or more of such compounds with at least one metallic element such as cupric sulphide with a metal of the chromium group—all have been successfully used as electronegative electrode materials. The electronegative electrode element 40 may consist of a mass of granular electronegative material or a solid body formed in any suitable and well known manner.
- In accordance with one modification of the 45 present invention the electropositive electrode element is preferably formed from pure magnesium, the surface of which may be oxidized in any suitable and well-known manner. The electronegative electrode element is preferably formed from a sulphide of copper or an alloy thereof, such as, for example, brass. This element 50 may be formed in the known manner of subjecting a metallic disc to the action of sulphur vapors or a sulphide of the metal may be formed, granulated and pressed into shape.
- In accordance with another modification of 55 the present invention, the electropositive electrode element may be formed from a silicon material, that is, silicon alone or a compound of silicon and an element chosen from an empirical group of more electropositive elements of the 60 electrochemical table of elements preferably chosen from the Second and Third Groups of Mendeleeff's Periodic Table of Elements, comprising beryllium, magnesium, calcium, zinc and aluminum. This electropositive electrode element is placed in surface contact with an electronegative electrode element having a high contact resistance with the electropositive electrode element and is preferably formed from, or provided with, a surface of a compound of an element 65 chosen from an empirical group of elements of Sub-Group B of the Sixth Periodic Group in Mendeleeff's Table of Elements, comprising sulphur, selenium and tellurium, or a mixture of such compounds. The other constituents of the 70 compound or compounds forming the electro-

negative material may be of any suitable metal or alloy thereof chosen from an empirical group of metals or materials comprising copper, silver, brass and bronzes.

The electropositive electrode element is preferably formed from granular magnesium silicide. The best mesh for such material has been found to be between about 36 and 60. With a finer mesh it has been found that the contact resistance is undesirably high and with a coarser mesh the resultant units are found to be undesirably leaky due to localized pressure. The electronegative electrode material in many instances is formed from granular cupric sulphide but a more preferable material is a mixture of cupric sulphide and 15 cupric selenide of about 100 mesh. A suitable method of forming such a mixture is by adding about 20 per cent selenium to the cupric sulphide and then heat treating the mixture for a considerable period of time, for example, about three 20 hours, at about 250° C. in a vacuum to prevent oxidation and to volatilize any excess of sulphur and selenium.

With such electropositive and electronegative materials, it is necessary to use a structure which 25 will confine these granular materials adjacent each other with sufficient pressure to insure good contact therebetween. This is readily accomplished by using a cup-shaped member in which the electropositive material in granular form is 30 placed over a mass of the electronegative material.

Any of the above described unilateral conductive couples are improved, in accordance with the present invention, by the use of a substance or substances tending to prevent, in operation, the 35 formation of polarizing material adjacent the electronegative material. It has been observed, in the operation of certain couples, that a rather common progressive decrease in the output occurs with an attendant decrease in efficiency, 40 which apparently is largely dependent upon the formation of an undesired layer of polarizing material adjacent the electronegative material. By providing a layer of non-polarizing substance adjacent the electronegative material in accordance 45 with the present invention, it has been found that the service life of any of such couples may be greatly increased. This having been determined, such couples are provided with such a layer of non-polarizing substance and may be efficiently 50 operated at a substantially constant output for a greatly increased service life. Examples of some of the more desirable non-polarizing substances are aquadag, carbon, graphite, tin, carbonized nickel, carbonized lead, alloys of nickel and chromium known under the trade name of "nichrome", and conductive carbides of relatively low resistance such as tungsten carbide, tantalum carbide and chromium carbide.

A layer of non-polarizing substance is preferably provided in the assembly in the following manner. A carbonized nickel element is inserted adjacent the electro-negative material, preferably in the shape of a washer. This washer constitutes 65 a sheet of nickel having a coating of carbon formed thereon. For the carbonized nickel may be substituted carbonized lead, that is a lead washer coated with carbon. Such an element is placed in the assembly with the carbonized side 70 adjacent the electronegative material. When conductive carbides of relatively low resistance are used, discs are formed from pressed powders thereof. When alloys of nickel and chromium known under the trade name of "nichrome" are 75

used a "nickrome" material having a relatively large amount of chromium is selected.

It has been found that thin sheets of brass containing about 20 per cent or more zinc may be used to prevent the formation of polarizing material adjacent the electro-negative electrode element provided that the rectifier assembly is kept under high pressure and the operating temperatures are kept below 150° C. Under such conditions these sheets of brass may be considered to be layers of non-polarizing material.

Referring to the drawing, Figs. 1 and 2 show structural embodiments of one form of the device of the present invention in which an elemental unilateral conductive couple of the dry surface-contact variety consists of an electropositive electrode element 10 of any suitable electropositive material, such as, for example, aluminum, magnesium, or an alloy or amalgam thereof, etc. This electrode element is preferably in the form of a washer and lies in face engagement with the electronegative electrode element 11 of any suitable electronegative material, such as, cupric sulphide, or a sulphided brass body. A layer 12 of non-polarizing substance is placed in contact with the opposite face of the electronegative electrode element 11. When these elements are in the form of washers they may be readily assembled as depicted in Fig. 2. Upon a bolt 13 provided with an insulating collar 14, and a pair of shoulder washers 15 and 16, is mounted a terminal plate 17 in face engagement with the electropositive electrode element 10 adjacent which is disposed the electronegative electrode element 11 in face engagement with the layer of non-polarizing substance 12. The layer 12 of non-polarizing substance engages another terminal plate 18 adjacent which is mounted another unilateral conductive couple, the non-polarizing layer 12 of which engages a third terminal plate 19. By the use of a bolt, means are provided for imposing pressure upon the elements to insure efficient contact therebetween.

In Fig. 3 is shown a structural modification preferably used when the electropositive and electronegative materials are in granular form. A base member 20, preferably in the shape of a disc or square sheet formed from copper, is provided with a threaded shank 21 and a projecting portion 22 serving as a terminal member. On the face of the projecting portion 22 is preferably disposed a washer 23 of lead and a thin sheet of carbonized nickel 24. A collar 25 is positioned over the projecting portion 22 to cooperate with the lead washer 23 and carbonized nickel element 24 and form a cup member having insulating walls 26 and a bottom provided with a layer of non-polarizing substance. The collar 25 may be formed from any suitable insulating material such as a vitreous enamel or magnesium silicate known to the trade as "steatite" and "lavite", but is preferably formed from aluminum and coated on the inside with an insulating oxide layer 26.

A mass 27 of granular electronegative material, preferably a mixture of copper sulphide and copper selenide, particles of which are preferably of about 100 mesh, is placed in the collar 25 over the layer of non-polarizing substance 24. A mass of electropositive material, such as magnesium silicide in granular form, the particles of which are of a size which will pass through a screen of between about 36 mesh and 60 mesh, is positioned over the mass 27 of electronegative material within the collar 25. Another lead washer 23' is placed over the electropositive ma-

terial 28 with, if desired, an interposed element 24' of plain nickel to prevent the grains of electropositive material from biting into the relatively soft surface of the lead washer 23' when pressure is applied. Another base member 20', having a threaded shank 21' and a projecting portion 22', serving as the other terminal member, is positioned as shown with the face of the projecting portion 22' in contact with the lead washer 23' within the collar 25. A resilient spider 29, having the arms thereof bowed as shown, is positioned over the shank 21' and bolts 30 extending through holes in the arms of the spider 29 and the base members 20 and 20' complete the assembly. The bolts 30 are provided with suitable insulating collars 31 to prevent short-circuiting of the asymmetric couple. An electrical terminal 32 is mounted upon the base member 20. The unit may be completed by mounting an additional electrical terminal 32' on the unit electrically connected with the base member 20' or, when these units are desired to be arranged in series, by coupling together shank 21' with the shank 21 of an adjacent unit by an internally threaded collar 33.

In Fig. 4 is shown a structural modification of the device depicted in Fig. 3 with four unilateral conductive couples arranged to change alternating current to direct current. Each couple consists of a pair of base members 34 and 34', preferably of copper and provided with plugs or projecting portions 35 and 35' adapted to serve as terminal members of the couple. Plugs 35 and 35' extend through the base members 34 and 34' respectively to form projections 36 and 36'. Adjacent couples have their base members 34, 34' electrically connected together by a metallic sleeve 37 which receives the projections 36', 36 as shown. Each couple is completed by a unit 38 which includes the electropositive and electronegative electrode elements, one of which is electrically connected to the plug 35 and the other of which is electrically connected to plug 35'.

The couples are preferably mounted in banks of two and secured together by bolts 39, 39, passing through end blocks 40, 40, preferably of steel so that the couples may be kept under desired pressure. The bolts 39, 39 may, if desired, pass through apertures in the base members 34, 34' since the latter are preferably made with a large surface area to act as efficient heat dissipating fins. In such case insulating sleeves 41, 41 are mounted on the bolts 39, 39 to eliminate the possibility of the couples being short-circuited by the bolts 39, 39. The end blocks 40, 40 are apertured to receive the projections 36, 36 and at least between one end block 40 and the adjacent base member 34 a shim 42 is mounted to allow the end block 40 to be resiliently stressed. The base members 34, 34 are provided with brackets 43, 43 to serve as supports and electrical connections.

As shown in Fig. 4, two banks are mounted side by side on metallic strips 44 and 45 which serve as electrical connectors between adjacent banks. The resultant structure is used to change alternating current to direct current by connecting the alternating current terminals 46 and 47 to the metallic strips 44 and 45, the direct current being delivered from the assembly by direct current terminals 48 and 49, one connected to a base member 34' in one bank and the other connected to a base member 34' in the other bank.

The couple unit 38 depicted in Fig. 6 is generally similar to that depicted in Fig. 3. It in-

cludes a collar 50 of insulating material such as magnesium silicate commercially known as "steatite" and "lavite" surrounded by a metallic ring 51 preferably of brass adapted to strengthen in the collar 50 and to serve as a heat dissipator. An additional feature of the unit 38 is the provision of a welded junction which increases the operating efficiency, avoids the necessity of a forming period when the unit is put in operation, and results in a unitary structure which can be readily handled.

The welded junction is preferably obtained by placing the collar 50 over a projecting electrode and inserting therein a lead washer 23, preferably about 30 mils thick, a carbonized nickel disc 24, preferably about one mil thick, a small amount of electronegative material, preferably a mixture of cupric sulphide and cupric selenide of about 100 mesh, a suitable amount of magnesium silicide, preferably between about 36 and 60 mesh, a nickel disc 24' and an additional lead washer 23' in the order set forth. A second electrode is brought into contact with the lead washer 23', pressure is applied, and current at a voltage and amperage greater than that at which the couple is designed to operate is allowed to flow between the electrodes from the electronegative material or anode side to the electrorespective material or cathode side. This flow of current is continued until the materials are welded together. As an example, welded junction couples designed to deliver about 5 amperes direct current at about 7 volts have been formed by placing them in a direct current circuit containing a variable resistance adjusted to allow about 50 amperes at about 12 volts to flow through the couple for periods of about 2 seconds each, these being repeated until the current flow was about 30 amperes. The resistance was then increased until the current flow was about 18 to 20 amperes and several 5-second periods of flow used until the voltage reached a maximum. Obviously, however, the production of welded junctions is not dependent upon the practice of the particular method described.

The use of at least one lead washer 23 adjacent the element 24 of non-polarizing substance is preferred in the assemblies since when sufficient pressure is applied to a couple unit the lead washer will be expanded to close completely the end of the collar 25 or 50 and seal off from the atmosphere the relatively unstable electronegative material. To insure efficient sealing a second lead washer 23' is used adjacent the electropositive material as shown.

The pressure used in the formation of welded junctions not only insures good contact between the electropositive and electronegative materials to obtain an efficient weld and formation of a current-blocking film but also expands the lead washers to seal off the electrode materials.

Pressure is additionally used in the completed assemblies to insure good contact between the adjacent surfaces of the elements, to allow the efficient formation at the junctions between the electropositive material and the electronegative material of an inverse current-blocking film when welded junctions are not used, to insure the maintenance of the current-blocking film during the operation of the device, and to allow rapid dissipation of heat.

In the operation of the device depicted the electropositive material forms the cathode and the electronegative material forms the anode and, when current is passed between these elec-

trode elements during the forming period, an inverse current-blocking film is formed therebetween. It is believed, but it is by no means certain that this current-blocking film when the anode is of copper sulphide and the cathode is of magnesium silicide, is a sulphide of silicon and magnesium. I do not wish, however, to be bound by this theory with regard to the probable nature of the compounds comprising the inverse current-blocking film.

The use of the non-polarizing substance, such as carbon, apparently prevents in operation the formation of polarizing material adjacent the electronegative material which has been found progressively to decrease the output of the asymmetric or unilateral conductive couple with a consequent decrease in efficiency and a relatively short service life.

It will thus be seen that the present invention efficiently attains the objects set forth above and provides asymmetric or unilateral conductive couples which are simple and rugged in structure and efficient in operation, units including electropositive electrode elements of a silicide of magnesium and electronegative electrode elements of an electronegative material including a sulphide of copper with which is associated a layer of a non-polarizing substance such as carbon having been operated continuously for periods greater than 1500 hours at a current density of about 100 amperes per square inch and 10 volts potential per couple without any appreciable decrease in the output.

The use of the expression "non-polarizing substances" is intended to cover all substances of the type set forth above which have the property in unilateral conductive couples of preventing the formation in operation of materials adjacent the electronegative material which develop during operation and decrease the output of the couple.

Since certain changes may be made in the above construction and different embodiments of the invention could be made without departing from the scope thereof, it is intended that all matter contained in the above description or shown in the accompanying drawing shall be interpreted as illustrative and not in a limiting sense.

Having described my invention, what I claim as new and desire to secure by Letters Patent, is:

1. In electric current rectifiers and the like, of the dry surface-contact variety, a relatively electropositive electrode element of magnesium, a relatively electronegative electrode element including a sulphide of copper in surface contact with said electropositive electrode, and a non-polarizing element of carbonized nickel in contact with said electronegative electrode element.

2. A unilateral conductive couple comprising a mass of silicide of magnesium maintained in contact with an electronegative material including a sulphide of copper, and a layer of non-polarizing substance in contact with said electronegative material.

3. A unilateral conductive couple comprising a mass of silicide of magnesium maintained in contact with a mixture of a sulphide of copper and a selenide of copper, and a non-polarizing element of carbonized nickel in contact with said mixture.

4. In electric current rectifiers and the like, of the dry surface-contact variety, a unilateral conductive couple comprising a relatively electropositive electrode element formed from one of

the materials beryllium, magnesium, calcium, zinc, aluminum, silicon and silicide, another electrode element having a surface of a relatively electronegative material of a compound of one of the elements sulphur, selenium and tellurium with one of the materials copper and copper alloys in surface-contact with said electropositive electrode and a non-polarizing element of carbonized nickel in contact with said electro-negative electrode element.

5. In electric current rectifiers and the like of the dry surface-contact variety, a unilateral conductive couple comprising a relatively electropositive electrode element formed from one of the materials beryllium, magnesium, calcium, zinc, aluminum, silicon and silicide, another electrode element having a surface of a relatively electronegative material of a compound of one of the elements sulphur, selenium and tellurium with one of the materials copper and copper alloys in surface contact with said electropositive electrode adapted to cooperate with the former for the electrochemical formation and maintenance of an inverse current-blocking film at their junction, and a layer of non-polarizing carbon containing material in contact with said electronegative material.

6. In electric current rectifiers and the like, of the dry surface-contact variety, a unilateral conductive couple comprising a relatively electropositive electrode element formed from one of the materials beryllium, magnesium, calcium, zinc, aluminum, silicon and silicide, another electrode element having a surface of a relatively electronegative material of a compound of one of the elements sulphur, selenium, and tellurium with one of the materials copper and copper alloys in surface contact with said electropositive electrode adapted to cooperate with the former for the electrochemical formation and maintenance of an inverse current-blocking film at their junction, and a non-polarizing element comprising a metal disc having a carbonized surface in contact with said electronegative material.

7. In electric current rectifiers and the like, of the dry surface-contact variety, a unilateral conductive couple comprising a relatively electropositive electrode element formed from one of the materials beryllium, magnesium, calcium,

zinc, aluminum, silicon and silicide, another electrode element of a relatively electronegative material formed from a compound of one of the elements sulphur, selenium and tellurium with one of the materials copper and copper alloys, 5 said electronegative body adapted to cooperate with the electropositive body for the electrochemical formation and maintenance of an inverse current-blocking film at their junction, and a non-polarizing element in contact with said 10 electronegative electrode, said non-polarizing element comprising one of the substances aquadag, carbon, graphite, tin, carbonized nickel, carbonized lead, tungsten carbide, tantalum carbide, chromium carbide and alloys of nickel and 15 chromium in which the amount of chromium preponderates.

8. In electric current rectifiers and the like, of the dry surface-contact variety, a unilateral conductive couple comprising a relatively electropositive electrode element formed from one of the materials beryllium, magnesium, calcium, zinc, aluminum, silicon and silicide, another electrode element of a relatively electronegative material formed from a compound of one of the elements sulphur, selenium and tellurium with one of the materials copper, brass and bronze, said electronegative body adapted to cooperate with the electropositive body for the electrochemical formation and maintenance of an inverse current-blocking film at their junction, and a non-polarizing element in contact with said 20 electronegative electrode, said non-polarizing element comprising one of the substances aquadag, carbon, graphite, tin, carbonized nickel, 25 carbonized lead, tungsten carbide, tantalum carbide, chromium carbide and alloys of nickel and chromium in which the amount of chromium 30 preponderates.

9. In electric current rectifiers and the like, of the dry surface-contact variety, a unilateral conductive couple comprising a relatively electropositive electrode member of magnesium, a relatively electronegative element including a sulphide of copper in surface contact with said electropositive electrode and a non-polarizing element having a carbon surface in contact with said electro-negative electrode element.

SAMUEL RUBEN.